

## UNITED STATES PATENT OFFICE

2,046,148

PROCESS FOR MANUFACTURING  
BERYLLIUM ALLOYS

Harry C. Clafin, Marysville, and James B. Arnold, St. Clair, Mich., assignors to The Beryllium Corporation, New York, N. Y., a corporation of Delaware

No Drawing. Application June 26, 1934,  
Serial No. 732,435

16 Claims. (Cl. 204—19)

This invention relates to a method for the direct manufacture of alloys of beryllium, in particular those of beryllium with copper, nickel, and iron.

5 Since the early work of Lebeau, in 1898, it has been known that the alloys of beryllium with copper and similar heavy metals have great value commercially, and more recent work has shown that the properties of such alloys are greatly enhanced by appropriate heat treatment. There has therefore been a great demand for such alloys, preponderant in the heavy metal, with beryllium content in the lower ranges—seldom over 5%.

15 The simple, laboratory method of alloy formation, direct fusion of the two metals, has been found, when transferred to a commercial scale, open to the objection that the losses are high and the cost of elementary beryllium metal is excessively high.

20 We have found that success can be attained readily if massive metal is used as a cathode electrode material; further, if this metal cathode is so suspended that any liquid alloy formed on its surface by the procedure of our invention can flow down readily away from the cathode into an electrically neutral area, operation can be made continuous, if desired.

25 In our invention, we suspend a massive cathode of the metal to be alloyed with beryllium in an electrolytic cell in which beryllium is being electrodeposited. As electrolyte in the cell, we may use any of those regularly in use for beryllium manufacture— $\text{BeCl}_2$  dissolved in  $\text{NaCl}$ ,  $\text{Na}_2\text{BeF}_4$ , 30 beryllium oxyfluoride dissolved in other fluorides, etc.; indeed, the process is essentially independent of the electrodeposition medium. The only requirement is that the bath (and, of course, with it the cathode) be maintained at a temperature below the melting point of the cathode but above that at which the lowest melting point (860° C. with copper) eutectic of the particular alloy which that metal forms with beryllium on electrolysis, melts. In the case of copper, as an 35 example, it is best to operate in the 900–1000° C. range; in this range the deposition of beryllium on the solid copper causes surface alloying which immediately causes the corresponding amount of alloy to turn liquid because of its lower melting point; this liquid will liquefy away from the electrode, baring new surfaces continuously. In this manner, and at this temperature range, a copper-beryllium alloy of about 2 to about 6% beryllium can readily be obtained.

40 For practical reasons, of course, it is best to

have two or more anodes for the cathode, but this is not at all necessary to the invention, though helping in actual practice to cause regular, even attack on the cathode. Attack on the cathode proceeds, we have found, with both a  $\text{BeCl}_2$  or a  $\text{Na}_2\text{BeF}_4$  bath, at a steady regular rate, a solid rod cathode merely tending to "pencil" as the electrolysis proceeds.

45 Naturally, as the newly-formed liquid alloy liquates away from the cathode of which it was just a part, it is brought to an electrically neutral—or primarily neutral—portion of the cell, so as to avoid counter-reactions. From this point (generally the bottom of the cell, away from both the cathode and the anode) the liquid alloy may readily be tapped away, either intermittently or, preferably, in continuous stream.

50 By combining this invention with that described in a co-pending application of H. C. Clafin, Serial No. 732,436, wherein there is described, a process for the production of beryllium in elementary or alloy form by the addition of ammonium beryllium fluoride to an alkali or alkaline earth metal fluoride bath and electrolyzed, we have attained a very convenient and effective procedure for the continuous production of commercial copper-beryllium alloys the electrolyzable salt being fed in continuously or at sufficiently frequent intervals, and the final alloy being also tapped off the cell continuously or at sufficiently frequent intervals.

55 In such procedure, there is nothing accumulating in the bath in that the fluorine and ammonium fluoride are evolved as gases and the beryllium tapped off in the alloy produced. Where the electrolyte is, for example,  $\text{Na}_2\text{BeF}_4$  there is a gradual accumulation of  $\text{NaF}$  in the bath, so that continuous operation cannot be so simply and economically obtained. Here it is necessary to remove a portion of the bath from time to time which involves a loss in values, and other objections. The periods of operation in such procedure must therefore be much shorter than possible when using ammonium beryllium fluoride, which may be months.

40 While copper has been used regularly as an example in the description given above, it can readily be seen that the process lends itself equally well to other metals with which beryllium alloys—most important commercially being iron and nickel.

45 In all cases, the metal salt or salts of the bath should be more electropositive than beryllium.

50 We also prefer to tap off the alloy from the cell in an atmosphere inert to beryllium or the

alloy, flowing the same into molds. This may be conveniently done, for example, by placing a hood over the cell and introducing an inert gas such as argon or helium. In such case, the tapping may be done by a rod insertable through the hood, especially if the pressure within the hood be kept slightly above atmospheric to avoid infiltration. Obviously, there may be a number of different ways in which the alloy may be tapped from the cell and kept out of contact with oxygen or nitrogen or other contaminant.

A further advantage in adding the beryllium in the form of ammonium beryllium fluoride is that the proportion of  $\text{BeF}_2$  in the bath can be raised above the point where "anode effect" objectionably sets in.

Having described our invention, we claim:

1. The process of forming alloys of beryllium characterized by the electrodeposition of beryllium on to an unmolten cathode of the second metal at a temperature below the melting point of that metal and above the melting point of the alloy eutectic.

2. The process of forming copper-beryllium alloys characterized by the electrodeposition of beryllium on to an unmolten copper cathode at a temperature below the melting point of copper and above the melting point of the copper-beryllium alloy eutectic.

3. The process of forming copper-beryllium alloys characterized by the electrolysis of electrolyzable beryllium compounds, using a cathode of massive copper, said electrolysis proceeding at a temperature between 860° C. and 1083° C.

4. The process of forming alloys of beryllium characterized by the electrodeposition of beryllium on to an unmolten cathode of the second metal at a temperature below the melting point of that metal and above the melting point of the alloy eutectic, the resultant fluid alloy being removed to an electrically neutral point.

5. The process of forming copper-beryllium alloys characterized by the electrodeposition of beryllium on to an unmolten copper cathode at a temperature below the melting point of copper and above the melting point of the copper-beryllium eutectic, the resultant fluid alloy being removed to an electrically neutral point.

6. The process of forming copper-beryllium alloys characterized by the electrolysis of electrolyzable beryllium compounds, using a cathode of massive copper, said electrolysis proceeding at a temperature between 860° C. and 1083° C., the resultant fluid alloy being removed to an electrically neutral point.

7. The process of forming alloys of beryllium characterized by the electrodeposition of beryllium on to an unmolten cathode of the second metal at a temperature below the melting point of that metal and above the melting point of the alloy eutectic, the resultant fluid alloy being removed, as formed, from the electrolytic field of action.

8. The process of forming copper-beryllium alloys characterized by the electrodeposition of beryllium on to an unmolten copper cathode at a temperature below the melting point of copper and above the melting point of the copper-beryllium eutectic, the resultant fluid alloy being removed, as formed, from the electrolytic field of action.

9. The process of forming copper-beryllium alloys characterized by the electrolysis of electrolyzable beryllium compounds, using a cathode of

massive copper, said electrolysis proceeding at a temperature between 860° C. and 1083° C., the resultant fluid alloy being removed, as formed, from the electrolytic field of action.

10. The process of forming alloys of beryllium characterized by the electrodeposition of beryllium on to an unmolten cathode of the second metal at a temperature below the melting point of that metal and above the melting point of the alloy eutectic, the resultant fluid alloy being removed, substantially as formed, from the electrolysis cell.

11. The process of forming copper-beryllium alloys characterized by the electrodeposition of beryllium on to an unmolten copper cathode at a temperature below the melting point of copper and above the melting point of the copper-beryllium alloy eutectic, the resultant fluid alloy being removed, substantially as formed, from the electrolysis cell.

12. The process of forming copper-beryllium alloys characterized by the electrolysis of electrolyzable beryllium compounds, using a cathode of massive copper, said electrolysis proceeding at a temperature between 860° C. and 1083° C., the resultant fluid alloy being removed, substantially as formed, from the electrolysis cell.

13. The continuous process of producing an alloy of beryllium and another metal or metals which consists in substantially continuously introducing an electrolyzable compound of beryllium into an electrolytic cell having a cathode of such metal or metals, operating at a temperature below the melting point of the cathode but above the melting point of the eutectic of the alloy formed, and in substantially continuously withdrawing the alloy produced.

14. The continuous process of producing an alloy of beryllium and another metal or metals which consists in substantially continuously introducing an electrolyzable compound of beryllium into an electrolytic cell having a cathode of such metal or metals, operating at a temperature below the melting point of the cathode but at which the alloy formed by the electrodeposition of the beryllium on the cathode liquates away, collecting the liquated alloy in an electrically neutral portion of the cell, and substantially continuously withdrawing such alloy.

15. The continuous process of producing an alloy of beryllium and another metal or metals which consists in substantially continuously introducing an electrolyzable compound of beryllium into an electrolytic cell having a cathode of such metal or metals, operating at a temperature below the melting point of the cathode but at which the alloy formed by the electrodeposition of the beryllium on the cathode liquates away, collecting the liquated alloy in an electrically neutral portion of the cell, and substantially continuously withdrawing such alloy in an atmosphere inert to the beryllium or the alloys.

16. The process of obtaining alloys of beryllium which includes the steps of adding ammonium beryllium fluoride to a fusion of the fluorides of one or more metals more electropositive than beryllium, subjecting the mixed fusion to electrolysis, using a cathode of the metal about to be alloyed with the beryllium and operating at a temperature substantially below the melting point of the cathode and above the melting point of the eutectic of the beryllium-metal alloy.

HARRY C. CLAFLIN.  
JAMES B. ARNOLD.